

Sept. 5, 1950

M. F. W. HEBERLEIN ET AL.  
ELECTROLYZING INDIUM OXIDE IN  
FUSED CAUSTIC ELECTROLYTE  
Filed Nov. 6, 1945

2,521,217



INVENTORS.  
MAX F. W. HEBERLEIN  
NEVIN R. BIERLY.

BY

David Crotty & Neal  
their ATTORNEYS.

## UNITED STATES PATENT OFFICE

2,521,217

## ELECTROLYZING INDIUM OXIDE IN FUSED CAUSTIC ELECTROLYTE

Max F. W. Heberlein, Rahway, and Nevin R. Bierly, Avenel, N. J., assignors to The American Metal Company, Limited, New York, N. Y., a corporation of New York

Application November 6, 1945, Serial No. 627,014

7 Claims. (Cl. 204—71)

1

This invention relates to electrolysis of indium in a fused caustic electrolyte.

We have found that the usual methods employed for the reduction of other metal oxides are not satisfactory when applied to indium recovery. Tests with several carbonaceous reducing agents gave varying low yields as compared with yields of the process herein described.

The principal object of the invention is to provide a simple, efficient process for recovering indium from indium material by electrolysis employing a fused caustic electrolyte. More particularly, the object of the invention is to provide a simple and efficient process for electrolyzing indium oxide obtained by the practice of the Heberlein (co-inventor of this application) and Udin process disclosed in their copending application Serial No. 622,022, filed October 12, 1945. Other objects of the invention will be in part obvious and in part pointed out hereinafter.

The invention accordingly consists of the novel processes and steps of processes, specific embodiments of which are described hereinafter by way of example and in accordance with which we now prefer to practice the invention.

In accordance with our invention, indium oxide is reduced to metal by electrolysis in fused caustic alkali, such as sodium hydroxide. Our method has the particular advantage that it may be practised with substantially little or no metal losses. The electrolysis is preferably performed in a steel vessel serving as cathode and which may be heated externally. The anode is suspended in the center, preferably, and consists of a steel strip about  $\frac{1}{2}$ " thick by 4" wide and about 6" long. The reduced indium metal collects as a molten pool at the bottom of the vessel and can be tapped periodically through an outlet provided for this purpose.

The operation of the electrolysis is conducted in the following manner in accordance with our invention. A flow sheet forming part of the application shows the steps employed.

Sodium hydroxide flakes are melted down in the steel vessel, whereupon the indium oxide ( $\text{In}_2\text{O}_3$ ) is added to the mass. Electrolysis is conducted with a current of about 400 amperes. Under this condition, about 300 grams of indium oxide ( $\text{In}_2\text{O}_3$ ) are consumed per hour, the indium being liberated to the molten pool at the bottom of the cell as mentioned.

The temperature of the fused caustic soda-indium oxide bath should preferably be about 800° F. and during the electrolysis the temperature range should be maintained at about the

order of 750–850° F. The current density maintained should be about 2.5 to 7 amperes per square inch of anode surface.

In the operation of electrolysis, very little external heating is necessary because most of the heat required to keep the electrolyte molten once it is brought within the heating range is supplied by the electric current.

Indium oxide is periodically stirred into the electrolyte during the run. Although iron or steel is highly resistant to the corrosive attack of fused caustic soda, the electrolyte dissolves a considerable amount of both the anode and the cathode. During the electrolysis, sodium oxide ( $\text{Na}_2\text{O}$ ) tends to build up. This material does not melt below its sublimation temperature of 1275° C. (2327° F.). It reacts very slowly with water or steam at the operating temperature of the cell and for this reason it can not be readily reconverted to sodium hydroxide during the electrolysis. For this reason it is considered preferable to discard the electrolyte every 48 hours, employing the above-sized apparatus, and to continue with a new batch of sodium hydroxide.

25 The discarded electrolyte mixture of sodium hydroxide and sodium oxide was found to contain up to about 3% iron and up to approximately 7% indium.

30 Since the indium oxide is dissolved in the caustic soda as  $\text{Na}_2\text{O} \cdot \text{In}_2\text{O}_3$ , or  $\text{NaInO}_2$ , metallic sodium is deposited at the cathode and  $\text{In}_2\text{O}_3$  must be liberated at the anode. The reduction of the  $\text{In}_2\text{O}_3$  is then brought about according to the following equation:



Some metallic sodium escapes this reaction, alloys with indium and collects in the metal pool in the bottom of the cell.

40 The product of the cell is a sodium-indium alloy containing up to 3–5% sodium. It has a melting point of approximately 725–750° F.

The metal which has been tapped from the cell is then transferred to a small gas-fired steel kettle for a final refining treatment. A typical spectrographic analysis of the metal tapped from the cell shows that it contains lead, tin, copper, iron, zinc, cadmium, sodium, with traces of antimony, thallium and bismuth, and the balance indium. This material is melted down in the kettle and the sodium is removed completely by pouring water onto the surface of the molten metal. Caustic soda forms and is skimmed off. The metal is then heated to about 600° F. and treated with caustic soda, water and niter for

the elimination of zinc and iron. Copper and a portion of tin are also removed with this treatment.

The caustic soda slag, together with the dross obtained by the above treatment with caustic soda, water and niter for the elimination of zinc and iron, are combined with the spent electrolyte. This material is then leached in hot water to separate the insoluble  $\text{In(OH)}_3$ , indium hydroxide, and the metallic indium prills. While the metallic prills are combined with the metal produced in the electrolytic cell, the indium oxide is returned to the operation for recovering indium and other values by combining it with the water leach residue to be supplied to the neutral leach, disclosed in the said copending application of Max F. W. Heberlein and Harry Udin. This indium hydroxide contains also other impurities such as iron and zinc, together with copper and small amounts of other metals or metal compounds resulting from the spent electrolyte and drosses formed.

An over-all indium recovery of 82% or better has been obtained by the practice of the process. The remaining indium is returned as indicated to the Heberlein and Udin process for further recovery.

The following constitute examples of the process as we now prefer to practise it. It is understood that the examples are illustrative and that the invention is not to be considered as restricted thereto except as indicated in the appended claims.

#### Example 1

About 18.5 kgs. of commercial sodium hydroxide flakes were melted down in a steel vessel of about 7' x 10' x 12" depth serving as a cathode which may be heated externally. This quantity of caustic soda gives a bath depth of approximately 10 inches. About 1.5 kgs. of indium oxide ( $\text{In}_2\text{O}_3$ ) containing a little  $\text{ZnO}$  are added to the molten bath and the temperature of the fused caustic soda-indium oxide bath is adjusted to about 800° F. A steel strip anode was then inserted in the molten bath. The steel anode consisted of a strip about  $\frac{1}{2}$ " thick and 4" wide. It was submerged in the center of the cell to about 4 inches from the bottom. Current of 400 amperes was used, giving a current density of about 7 amperes per square inch anode surface. The temperature of the bath was maintained at about 750-850° F. The initial cell voltage was approximately 5 volts. After about 48 hours it increased to nearly 7.5 volts. Most of the heat required to keep the electrolyte molten was supplied by the current. About 150 grams of indium oxide ( $\text{In}_2\text{O}_3$ ) were added every half hour. Larger quantities tended to thicken the electrolyte too much for smooth operation in the particular apparatus employed. Under this condition about 300 grams  $\text{In}_2\text{O}_3$  were consumed per hour. The reduced indium metal, an alloy of indium and sodium, melting at 725-750° F., collected as a molten pool in the bottom and was tapped periodically from an outlet provided for that purpose.

During the course of the electrolysis, sodium oxide ( $\text{Na}_2\text{O}$ ) which does not melt below the sublimation temperature of 1275° C. (2327° F.), collects in the cell. It reacts very slowly with water and steam at the operating temperatures of the cell and for this reason it was not converted to caustic soda during the electrolysis. At the end of every 48 hours the electrolyte which had built up a certain quantity of iron and sodium oxide,

was removed and replaced by a batch of 18.5 kgs. of fresh fused sodium hydroxide.

The electrolyte mixture of sodium hydroxide-sodium oxide containing up to 3% iron and up to approximately 7% indium upon removal from the cell was then leached in hot water to separate the insoluble indium hydroxide  $\text{In(OH)}_3$  and metallic indium prills. The metallic prills were combined with the metal produced in the electrolytic cell, the indium hydroxide being returned to the operation by combining it with the residue resulting from the acid leach of the water leach residue as described in the copending application of Max F. W. Heberlein and Harry Udin, Serial No. 622,022, filed October 12, 1945. The following shows the metal balance of a run of 48 hours using the single cell operation described:

|                                         | Kgs. |
|-----------------------------------------|------|
| $\text{In}_2\text{O}_3$ charged to cell | 14.0 |
| In-content of charge                    | 11.2 |
| In-content of spent electrolyte         | 2.1  |
| Metal tapped from cell                  | 9.0  |
| Loss                                    | 0.1  |

25 The metal tapped from the cell was remelted in a gas-fired steel kettle for a final refining treatment. Spectrographic analysis of the metal tapped from the cell is shown in the following:

|    |           |    |           |
|----|-----------|----|-----------|
| Pb | .05%      | Zn | High>0.5% |
| Sn | .04%      | Tl | Trace     |
| Sb | Trace     | Cd | .005%     |
| Cu | .005-.02% | Na | High>1.0% |
| Fe | .02-.04%  | In | Balance   |
| Bi | Trace     |    |           |

25 This material is melted in the kettle and the sodium is removed completely by water poured onto the surface of the molten metal. A viscous caustic soda slag forms and can be easily skimmed off. The metal is then heated to about 600° F. and treated with caustic soda, water and niter ( $\text{NaNO}_3$ ) for the elimination of zinc and iron as oxides. A typical assay of the refined metal shows the following impurities:

|    |       |    |              |
|----|-------|----|--------------|
| Pb | .04%  | Tl | Trace        |
| Sn | Trace | Bi | Trace        |
| Sb | Trace | Fe | .01%         |
| Cu | .005% | Na | Not detected |
| Zn | Trace | In | Balance      |
| Cd | Trace |    |              |

30 The kettle treatment result as follows:

|                                | Kgs.  |
|--------------------------------|-------|
| Cell metal charged to kettle   | 38.54 |
| Metal heel from previous batch | 3.57  |
| Total charge                   | 42.11 |

|                                         |       |
|-----------------------------------------|-------|
| Refined metal cast from this charge     | 38.57 |
| Metal-In and Na and impurities to dross | 3.54  |

35 The kettle dross resulting from the above is combined with hot spent electrolyte and leached in hot water. The residue consisting mostly of indium hydroxide is returned to the neutral leach operation of the Heberlein and Udin process mentioned above.

#### Example 2

40 About 18.5 kgs. of commercial sodium hydroxide flakes were charged into each of two steel cells connected electrolytically in series, the dimensions of the cells being substantially those mentioned in Example 1. To each of the molten baths in these cells was added 1.5 kgs. of indium oxide ( $\text{In}_2\text{O}_3$ ) containing a little  $\text{ZnO}$  and the

temperature of the fused caustic soda-indium oxide bath is adjusted in each cell to about 800° F. A steel strip of the dimensions given in Example 1 was inserted in each cell in the manner described in Example 1. Electrolysis was conducted employing a current of about 400 amperes and a current density of about 7 amperes per square inch of anode surface. The operation was conducted for 48 hours in substantially the same manner as that in Example 1 and the results are shown in the following metal balance:

|                                                | Kgs. |
|------------------------------------------------|------|
| In <sub>2</sub> O <sub>3</sub> charged to cell | 27.8 |
| In-content of charge                           | 22.2 |
| In-content of spent electrolyte                | 5.8  |
| Metal tapped from 2 cells                      | 16.3 |
| Loss                                           | 0.1  |

We claim:

1. The process which essentially comprises, electrolyzing indium oxide (In<sub>2</sub>O<sub>3</sub>) containing iron as impurity dissolved in molten sodium hydroxide at a temperature of about 750-850° F. to produce impure indium metal, thereby building up the content of sodium oxide and iron in the electrolyte, and recovering said impure indium metal.

2. The process which essentially comprises electrolyzing indium oxide (In<sub>2</sub>O<sub>3</sub>) dissolved in molten caustic alkali to form a sodium-indium alloy, maintaining the temperature of the bath at a point where the alloy collects as a molten mass, removing the alloy, and recovering the indium.

3. The process which essentially comprises electrolyzing indium oxide (In<sub>2</sub>O<sub>3</sub>) dissolved in molten sodium hydroxide to form a sodium-indium alloy, using as electrodes a metal of a high melting point, maintaining the temperature of the bath at a point where the alloy collects as a molten mass, removing the alloy, and recovering the indium.

4. The process which essentially comprises electrolyzing indium oxide (In<sub>2</sub>O<sub>3</sub>) dissolved in molten caustic alkali to form a sodium-indium alloy, using steel electrodes, maintaining the temperature of the bath at 750-850° F., removing the alloy, and recovering the indium.

5. The process which essentially comprises electrolyzing indium oxide (In<sub>2</sub>O<sub>3</sub>) dissolved in molten sodium hydroxide to form a sodium-in-

dium alloy, maintaining the temperature of the bath at a point where the alloy collects as a molten mass, adding water to said alloy, and removing a dross containing sodium hydroxide.

5 6. The process which essentially comprises electrolyzing indium oxide (In<sub>2</sub>O<sub>3</sub>) dissolved in molten caustic soda to form a sodium-indium alloy containing small amounts of sodium, iron and zinc, adding water to the alloy, removing a dross containing sodium hydroxide, treating the resultant metal after removal of the sodium hydroxide with niter, sodium hydroxide and water to form a dross containing iron and zinc and removing the last-mentioned dross.

10 15 7. The process which essentially comprises electrolyzing indium oxide (In<sub>2</sub>O<sub>3</sub>) containing iron and zinc as impurities dissolved in molten sodium hydroxide at a temperature of about 750-850° F. to form a pool of impure indium metal containing sodium, iron and zinc, removing spent electrolyte when the iron content thereof reaches about 3%, oxidizing sodium, iron and zinc contained in the impure metal, removing such oxidized metals from said indium metal, 20 and recovering indium values from the spent electrolyte and said oxidized metals.

MAX F. W. HEBERLEIN.  
NEVIN R. BIERLY.

#### REFERENCES CITED

30 The following references are of record in the file of this patent:

#### UNITED STATES PATENTS

| 35 Number    | Name                  | Date           |
|--------------|-----------------------|----------------|
| 785,962      | Lyons et al. -----    | Mar. 28, 1905  |
| 1,338,279    | Blumenberg -----      | Apr. 27, 1928  |
| 2,238,437    | Zischkau -----        | Apr. 15, 1941  |
| 2,241,438    | Zischkau et al. ----- | May 13, 1941   |
| 40 2,384,610 | Doran et al. -----    | Sept. 11, 1945 |

#### FOREIGN PATENTS

| Number  | Country      | Date          |
|---------|--------------|---------------|
| 163,812 | France ----- | Aug. 18, 1884 |

#### 45 OTHER REFERENCES

“Comptes Rendus,” vol. 190 (1930), pages 925-927.

“Metal Finishing,” July 1944, page 406.

50 “Transactions of The Electrochemical Society,” vol. 85 (1944), pages 223, 224.